# EUROPEAN PATENT APPLICATION

(11) **EP 4 342 598 A1**
(43) Date of publication of application: **27.03.2024**
(21) Application number: 23193050.4
(22) Date of filing: 23.08.2023
(51) Int. Cl.: B21H 1/14, B21B 1/085, B21B 1/16, B21K 1/02

(54) **METHOD OF ROLLING BALLS**

(30) Priority: 21.09.2022 PL 44234322
(71) Applicant: "Firma Codogni" Spolka Jawna, 37-464 Stalowa Wola (PL)
(72) Inventor: Tofil, Arkadiusz, 22-100 Chelm (PL); Tomczak, Janusz, Swidnik (PL); Krawiec, Damian, 21-107 Sawin (PL)
(74) Representative: AOMB Polska Sp. z.o.o.

(57) **Abstract**

A method of rolling balls, especially from webs of scrap railway rails, characterized in that a blank (17) in the shape of a web of a railway rail is heated to the temperature appropriate for hot forming, after which the heated blank (17) is placed in grooves (2a) and (2b) of feeding rolls (1a) and (1b), then the feeding rollers (1a) and (1b) are set to rotate at the same speed (n1) and the blank (17) is moved towards a front guide (3) at a constant speed (V1), thereafter, grooved rolls of a first stand (5a) and (5b) are set to rotate at a constant speed (n2) in opposite directions, and grooved rolls of a second stand (11a) and (11b) are set to rotate at a constant speed (n3) in opposite directions, at the same time, guide rollers (15a) and (15b) are set to rotate at a constant speed (n4) in the same direction, and, at the same time, helical rolls (20a) and (20b) are set to rotate at equal speeds (n5) in the same direction, thereafter the blank (17) is guided into a guide hole (4) of a front guide of the first stand (3) and the blank (17) is moved towards the grooved rolls of the first stand (5a) and (5b), and the blank (17) is guided into oval-shaped grooves (6a) and (6b) located on the surface of the grooved rolls of the first stand (5a) and (5b), which have a depth (h1) less than half the height of the blank (17) and a width (b 1) greater than the thickness of the blank (17), while the diameter (D1) of both grooved rolls of the first stand (5a) and (5b) is the same, wherein axes of the both grooved rolls of the first stand (5a) and (5b) are located in a horizontal plane, and the distance between the axes of the both grooved rolls of the first stand (5a) and (5b) is equal to the diameter (D1) of the grooved rolls of the first stand (5a) and (5b).

## Description

The invention relates to a method of rolling balls, especially from webs of scrap railway rails.

A number of methods for manufacturing balls intended for grinding media for ball mills have been known and used so far. The most common ones include casting, die forging and rolling. The balls are cast from cast steel which is cast into permanent moulds made of metal, the so-called casting dies. Die forging of balls is typically carried out on friction presses, with the use of billets in the form of bars made of steel with increased carbon and manganese content. Immediately after the forging process, the flash is trimmed on eccentric presses. The highest efficiency in the production of balls is achieved using the skew rolling process. Information on the skew rolling of balls has been presented in a book by W. Dobrucki, "Zarys obróbki plastycznej metali" ("Outline of plastic forming of metals"), Wydawnictwo "Śl sk", Katowice, 1975. The process described in the book enables shaping of a single ball forging during one rotation of the rolls. During one minute, 160 balls with a diameter of about Ø 30 mm or 40 balls with a diameter of about Ø 120 mm are obtained. The balls are rolled in skew rolling mills equipped with two rolls with helically cut single grooves, typically 3.5 turns in length. The axes of the rolls are inclined obliquely to the axis of the billet - a bar, at an angle of 3° to 7°. During rolling, the rolls rotate in the same direction, while the billet rotates in the opposite direction. To obtain good rolling results, the diameter of the billet should be about 0.97 of the diameter of the finished balls, while the diameter of the rolls should be 5 to 6 times greater than the diameter of the rolled balls. Also known and used are methods of processing scrap railway rails, which allow for management of the railway scrap and obtaining a valuable consumable material from it. The most common methods include die forging of blanks from sections of heads of scrap railway rails and longitudinal rolling of bars from heads cut off from worn rails. The processes of longitudinal rolling of circular cross-section bars from the heads of scrap railway rails are described in detail in a book by Z. Pater, J. Tomczak, "Walcowanie śrubowe kul do m ynów kulowych" ("Helical rolling of balls for ball mills"), Wydawnictwo Politechniki Lubelskiej, Lublin 2012. Depending on the diameter of the bars, the rolling process presented in the book is carried out between two or four pairs of rolls with parallel axes that rotate in opposite directions. The surfaces of the rolls have oval and circular groove cuts. In the first pass, a section of the head of the scrap railway rail is rolled in an oval cut, then the blank in the form of an oval-shaped bar is transferred to the second - circular cut, where the bars with a circular cross-section are rolled. In the case of forging rolling, the length of billets used for rolling is limited by the possibility of feeding them into the workspace of the rolls and by their weight. Most often, in such a process, the billet is fed manually and is held in the tongs throughout the shaping process. The aforementioned limitation does not occur in the case of metallurgical rolling, which allows for shaping bars with a length of up to several meters. The authors indicate that it is also possible to roll bars with circular cross-section in skew rolling mills. In the skew rolling process, the rolls are arranged symmetrically around the blank, and their axes are twisted at equal angles to the rolling axis. During the rolling process, the tools rotate at constant speeds in the same direction, grabbing the blank and pulling it into the workspace, where the bars are rolled as a result of flow formation of the blank. The use of the skew rolling process to produce a round bar from the rail head requires that its end is shaped into a cone, which is necessary in view of a smooth introduction of the material between the rolls. In order to initiate the rolling process, it is also necessary to use a pusher, which is used to feed the blank between the rolls, which then, while shaping the bar, will automatically pull it into the space between the rolls.

Polish patent PL 225772 discloses a method of skew rolling of bars with circular cross-section from the heads of scrap railway rails. The method consists in shaping bars between two rolls, which in the initial part have flanges, gradually flow forming the material during the rotation. The method disclosed in the patent requires the use of two rolls with a complicated shape, further it is necessary to guide the material in the workspace between two strips, which significantly reduces the stability of the process. Another limitation of the technology is the need to use different sets of rolls depending on the diameter of the bars to be shaped.

Polish patent application No. P.423386 discloses also a method of rolling bars from webs of scrap railway rails, which consists in two-step rolling of bars. In the first step, a preform with a nearly hexagonal cross-section is rolled longitudinally in a groove cut. Subsequently, in the second step, such a blank is rolled in a skew rolling mill between three tools into a bar of circular cross-section. This method allows for manufacturing of geometrically and dimensionally accurate bars with a circular cross-section from webs cut off from worn railway rails in a fairly wide range of diameters. The limitation of this technology may be a relatively low efficiency of such rolling.

A characteristic feature of the currently known and used methods of rolling ball forgings is the need to use blanks in the form of bars with high geometrical and dimensional accuracy. As a result, it makes it necessary to use metallurgical bars as billets. However, no processes of skew rolling of balls are available, which would be carried out in a small number of cuts immediately after the longitudinal rolling of scrap elements.

The objective of the invention is to provide rolling of ball forgings directly from webs cut off from worn railway rails.

The essence of a method of rolling balls, especially from webs of scrap railway rails, according to the invention, is that a blank in the shape of a web of a railway rail is heated to the temperature appropriate for hot forming. After that, the heated blank is placed in grooves of feeding rolls, then, the feeding rollers are set to rotate at the same speed and the blank is moved towards a front guide at a constant speed. Thereafter, grooved rolls of a first stand are set to rotate at a constant speed in opposite directions, and grooved rolls of a second stand are set to rotate at a constant speed in opposite directions, at the same time, guide rollers are set to rotate at a constant speed in the same direction, and, at the same time, helical rolls are set to rotate at equal speeds in the same direction. After that, the blank is guided into a guide hole of a front guide of the first stand and the blank is moved towards the grooved rolls of the first stand, and the blank is guided into an oval-shaped grooves located on the surface of the grooved rolls of the first stand, which have a depth less than half the height of the blank and a width greater than the thickness of the blank, and the diameter of the both grooved rolls of the first stand is the same. The axes of the both grooved rolls of the first stand are located in a horizontal plane, and the distance between the axes of the both grooved rolls of the first stand is equal to the diameter of the grooved rolls of the first stand. The blank is then gripped with groove surfaces of the grooved rolls of the first stand and the blank in the shape of the railway rail web is flow formed into an oval-shaped blank. The vertical axis of an oval cut formed by the grooves of the grooved rolls of the first stand has a length which is greater than the length of the horizontal axis of the oval-shaped cut formed by the grooves of the grooved rolls of the first stand, wherein an oval-shaped blank is held in the rolling axis behind a rolling gap of the grooved rolls of the first stand in an oval-shaped hole of a rear guide of the first stand. After that, the blank is moved towards the second rolling stand, which consists of two identical grooved rolls of the second stand, which have the same diameter and concave grooves on their surfaces, with a radius equal to half the diameter of the rolled ball, and the axes of the grooved rolls of the second stand are horizontal and are spaced apart by the diameter of the grooved rolls of the second stand. Then the end of the blank is guided into a hole of an entry guide of the second rolling stand, then the end of the blank is guided into circular-shaped grooves, which are located on the cylindrical surfaces of the grooved rolls of the second stand, and the blank with an oval-shaped cross-section is flow formed into a bar with a nearly circular cross-section. The diameter of the bar is greater than the diameter of the rolled ball. Behind the rolling gap of the second stand, the rolled bar is guided in a square-shaped hole of the rear guide of the second rolling stand.

The rolled bar is moved in grooves of the guide rollers in the direction of skew rolls and the bar is guided into a hole of a guiding sleeve, in which the correct position of the bar is maintained, then, using the guide rollers, the bar is guided into the workspace of a skew rolling mill, consisting of two helical rolls and two guides. Both helical rolls have the same working diameter, and their axes are twisted in opposite directions relative to the rolling axis by the same value of the twist angle of the rolls, and the guides are located parallel to the rolling axis, and the distance between the working surfaces of the guides is greater than the diameter of the rolled bar. After that, the end of the bar is gripped with conical surfaces located in an entry zone of the two helical rolls, which rotate with equal speeds in the same direction, the bar is set to rotate at a constant speed in the direction opposite to the direction of rotation of the helical rolls, and the cross-section of the bar is flow formed using conical surfaces and the cross-section of the bar is calibrated to a diameter smaller than the diameter of the rolled ball using two cylindrical surfaces located behind the conical surfaces of the helical rolls. Subsequently, helical protrusions located on the surfaces of the helical rolls are sunk into the cylindrical surface of the earlier calibrated bar. The helical protrusions of the helical rolls have concave side surfaces, the radius of which is equal to half the diameter of the rolled ball. Then, annular grooves with spherical side surfaces are gradually formed on the blank, the blank being held in a workspace during rolling by two guides, located opposite each other, between the helical rolls. Then, as a result of the action of the helical protrusions with concave side surfaces located on the helical rolls, the depth of the annular grooves increases until the ball is formed and completely separated from the bar. As a result, the ball with a diameter smaller than the diameter of the bar is obtained.

The advantageous effect of the invention is that it allows for plastic shaping of balls directly from a blank in the shape of a web section cut off from worn railway rails. As a result, it is possible to roll ball forgings with a minimum number of longitudinal stands. The invention is characterized by a high efficiency of ball production as compared with that achieved in the die forging and casting processes. Further, the use of bar calibration immediately before rolling of the balls shortens the rolling time and reduces the sensitivity of the process to the geometric accuracy of the blanks.

The invention is presented in an embodiment in the drawings, wherein Fig. 1 shows an isometric view of the rolling process in the initial stage, Fig. 2 shows an isometric view of the process during rolling of a bar in longitudinal stands, Fig. 3 shows an isometric view of the process after rolling of a bar, Fig. 4 shows an isometric view of the process during rolling of balls, Fig. 5 shows a side view of tools and rolled balls, fig. 6 shows the A-A section through the axis of the first stand, Fig. 7 shows the B-B section through the axis of the second stand, Fig. 8 shows the C-C section through the rolling axis in the skew stand.

A method of rolling balls, especially from webs of scrap railway rails, consists in that a blank 17 in the shape of a railway rail web was heated to the temperature appropriate for hot working, which was 1200°C. Then, the heated blank 17 was placed in the grooves 2a and 2b of the feeding rollers 1a and 1b. After that, the feeding rollers 1a and 1b were set to rotate at the same speed n1 of 60 rpm, and the blank 17 was moved towards the front guide 3 at a constant speed V1 of 100 mm/s. Subsequently, the grooved rolls of the first stand 5a and 5b were set to rotate at a constant speed n2 of 12 rpm in opposite directions. At the same time, the grooved rolls of the second stand 11a and 11b were set to rotate at a constant speed n3 of 16 rpm in opposite directions, and the guide rollers 15a and 15b were set to rotate at a constant speed n4 40 rpm in the same direction and at the same time the helical rollers 20a and 20b were set to rotate at the same speeds n5 of 40 rpm in the same direction. Then, the blank 17 was guided into a guide hole 4 of the front guide of the first stand 3, and the blank 17 was moved towards the grooved rolls of the first stand 5a and 5b, and the blank 17 was guided into the oval-shaped grooves 6a and 6b located on the surface of the grooved rolls of the first stand 5a and 5b. The grooves 6a and 6b of the grooved rolls of the first stand 5a and 5b had a depth h1 of 25 mm, which was less than half the height of the blank 17, and a width b1 equal to 19 mm which was greater than the thickness of the blank 17. The diameter D1 of both grooved rolls of the first stand 5a and 5b was the same and was 500 mm, and the axes of both grooved rolls of the first stand 5a and 5b were located in a horizontal plane, and the distance between axes of both grooved rolls of the first stand 5a and 5b was the diameter D1 of the grooved rolls of the first stand 5a and 5b, and was equal 500 mm. Then the blank 17 was gripped with the groove surfaces 6a and 6b of the grooved rolls of the first stand 5a and 5b and the blank 17 in the shape of a railway rail web was flow formed into an oval-shaped blank 17b. The vertical axis of the oval cut formed by the grooves 6a and 6b of the grooved rolls of the first stand 5a and 5b had a length 2h1 of 50 mm, which was greater than the length b1 of the horizontal axis of the oval cut formed by the grooves 6a and 6b of the grooved rolls of the first stand 5a and 5b. The oval-shaped blank 17b was held in the rolling axis behind the rolling gap of the grooved rolls of the first stand 5a and 5b in an oval-shaped hole 8 of the rear guide of the first stand 7. Then the blank 17b was moved towards the second rolling stand, which consisted of two identical grooved rolls of the second stand 11a and 11b, which had the same diameter D2 equal to 500 mm, and on their surfaces were concave grooves 12a and 12b with a radius R2 of 16.5 mm, which was equal to half the diameter dk of the rolled ball of 33 mm. The axes of the grooved rolls of the second stand 11a and 11b were located horizontally and spaced apart by the diameter D2 of the grooved rolls of the second stand 11a and 11b, equal to 500 mm. Thereafter, the end of the blank 17b was guided into a hole 10 of the entry guide 9 of the second rolling stand, after which the end of the blank 17b was guided into the circular-shaped grooves 12a and 12b, which were located on the cylindrical surfaces of the grooved rolls of the second stand 11a and 11b, and the blank 17b with a oval-shaped cross-section was flow formed into a bar 17c with nearly circular cross-section. The diameter dp of the bar was 33.5 mm and was greater than the diameter dk of the rolled ball 18 of 33 mm. Thereafter, behind the rolling gap of the second stand, the rolled bar 17c was guided in a square-shaped hole 14 of the rear guide 13 of the second rolling stand. Then the rolled bar 17c was moved in the grooves 16a and 16b of the guide rollers 15a and 15b towards the skew rolls 20a and 20b, and the bar 17c was guided into a hole of the feeding sleeve 19, in which the correct position of the bar 17c was maintained. Then, using the guide rollers 15a and 15b, the bar 17c was guided into the workspace of the skew rolling mill, consisting of two helical rolls 20a and 20b and two guides 24a and 24b. Both helical rolls 20a and 20b had the same working diameter D of 340 mm, and their axes were twisted in opposite directions relative to the rolling axis by the same twist angle of the rolls γ, which was 5°. The guides 24a and 24b were parallel to the rolling axis, and the distance between the working surfaces of the guides 24a and 24b was greater than the diameter dp of the rolled bar 17c, and during the rolling was equal to 35 mm. Then, the end of the bar 17c was gripped with conical surfaces 21a and 21b located in the entry zone of two helical cylinders 20a and 20b, which rotated at the same speeds n5 in the same direction, and the bar 17c was set to rotate at a constant speed n6 of 400 rpm in the direction opposite to the direction of rotation of the helical rolls 20a and 20b, and the bar 17c was moved at a speed V2 of 45 mm/s, and using the conical surfaces 21a and 21b the cross-section of the bar 17c was flow formed, by shaping a transitional conical surface with an opening angle α of 5°, and then the cross-section of the bar 17c was calibrated using two cylindrical surfaces 22a and 22b located behind the conical surfaces of the helical rolls 20a and 20b to a diameter d of 31.5 mm, which was smaller than the diameter of the rolled ball dk, which was 33 mm. Subsequently, helical protrusions located on the surfaces of the helical rolls 20a and 20b were sunk into the cylindrical surface of the earlier calibrated bar 17c. The concave side surfaces 23a and 23b of the helical protrusions of the helical rolls 20a and 20b had concave side surfaces 23a and 23b, the radius Rk of which was 16.5 mm and was equal to half the diameter dk of the rolled ball 18. Then, annular grooves with spherical side surfaces were gradually formed on the blank 17c. During the rolling, the blank was held in the workspace by two guides 24a and 24b, located opposite each other, between the helical rolls 20a and 20b. Then, as a result of the action of the helical protrusions with concave side surfaces 23a and 23b of the helical rolls 20a and 20b, the depth of the annular grooves was increased until the ball 18 was formed and completely separated from the bar 17c. As a result of the action of the helical projections with concave side surfaces 23a and 23b, a ball 18 with a diameter dk equal to 33 mm, smaller than the diameter dp of the bar 17c, equal to 33.5 mm, was formed.

### List of reference signs

- 1a, 1b: - feeding rollers
- 2a, 2b: - grooves on feeding rollers
- 3: - front guide of the first stand
- 4: - guide hole of the front guide
- 5a, 5b: - grooved rolls of the first stand
- 6a, 6b: - oval-shaped grooves
- 7: - rear guide of the first stand
- 8: - oval-shaped hole
- 9: - entry guide of the second stand
- 10: - hole of the entry guide of the second stand
- 11a, 11b: - grooved rolls of the second stand
- 12a, 12b: - circular-shaped grooves
- 13: - rear guide of the second stand
- 14: - square-shaped hole of the rear guide
- 15a, 15b: - guide rollers
- 16a, 16b: - grooves of guide rollers
- 17: - blank in the shape of a section of railway rail web
- 17b: - oval-shaped blank
- 17c: - blank with nearly circular cross-section
- 18: - rolled ball
- 19: - feeding sleeve
- 20a, 20b: - helical rolls
- 21a, 21b: - conical surfaces of helical rolls
- 22a, 22b: - cylindrical surfaces of helical rolls
- 23a, 23b: - concave surfaces of helical protrusions
- 24a, 24b: - guides
- 36: - rolled balls
- D: - diameter of helical rolls
- D1: - diameter of grooved rolls of the first stand
- D2: - diameter of grooved rolls of the second stand
- dk: - diameter of rolled ball
- dp: - diameter of rolled bar
- d: - diameter of calibrated bar
- h1: - depth of grooves of the grooved rolls of the first stand
- b1: - length of horizontal axis of the oval cut
- Rk: - radius of concave side surfaces of the helical protrusions
- R2: - radius of concave grooves of the grooved rolls of the second stand
- n1: - speed of guide rollers
- n2: - speed of grooved rolls of the first stand
- n3: - speed of grooved rolls of the second stand
- n4: - speed of guide rollers
- n5: - speed of helical rolls
- n6: - rotational speed of the bar
- V1: - speed of blank movement
- V2: - speed of bar movement
- α: - opening angle of conical surface
- γ: - twist angle of the axes of helical rolls

## Claims

1. A method of rolling balls, especially from webs of scrap railway rails, **characterized in that** a blank (17) in the shape of a web of a railway rail is heated to the temperature appropriate for hot forming, after which the heated blank (17) is placed in grooves (2a) and (2b) of feeding rolls (1a) and (1b), then the feeding rollers (1a) and (1b) are set to rotate at the same speed (n1) and the blank (17) is moved towards a front guide (3) at a constant speed (V1), thereafter, grooved rolls of a first stand (5a) and (5b) are set to rotate at a constant speed (n2) in opposite directions, and grooved rolls of a second stand (11a) and (11b) are set to rotate at a constant speed (n3) in opposite directions, at the same time, guide rollers (15a) and (15b) are set to rotate at a constant speed (n4) in the same direction, and, at the same time, helical rolls (20a) and (20b) are set to rotate at equal speeds (n5) in the same direction, thereafter the blank (17) is guided into a guide hole (4) of the front guide of the first stand (3) and the blank (17) is moved towards the grooved rolls of the first stand (5a) and (5b), and the blank (17) is guided into oval-shaped grooves (6a) and (6b) located on the surface of the grooved rolls of the first stand (5a) and (5b), which have a depth (h1) less than half the height of the blank (17) and a width (b1) greater than the thickness of the blank (17), while the diameter (D1) of both grooved rolls of the first stand (5a) and (5b) is the same, wherein axes of the both grooved rolls of the first stand (5a) and (5b) are located in a horizontal plane, and the distance between the axes of the both grooved rolls of the first stand (5a) and (5b) is equal to the diameter (D1) of the grooved rolls of the first stand (5a) and (5b), then the blank (17) is then gripped with the groove surfaces (6a) and (6b) of the grooved rolls of the first stand (5a) and (5b), and the blank (17) in the shape of the web of the railway rail is flow formed into an oval-shaped blank (17b), wherein a vertical axis of an oval cut formed by the grooves (6a) and (6b) of the grooved rolls of the first stand (5a) and (5b) has a length (2h1) which is greater than the length (b1) of the horizontal axis of the oval cut formed by the grooves (6a) and (6b) of the grooved rolls of the first stand (5a) and (5b), wherein the oval-shaped blank (17b) is held in the rolling axis behind the rolling gap of the grooved rolls of the first stand (5a) and (5b) in an oval-shaped hole (8) of a rear guide (7) of the first stand, after which the blank (17b) is moved towards the second rolling stand, which consists of two identical grooved rolls of the second stand (11a) and (11b), which have the same diameter (D2) and concave grooves (12a) and (12b) on their surfaces, with a radius (R2) equal to half the diameter (dk) of a rolled ball (18), and the axes of the grooved rolls of the second stand (11a) and (11b) are horizontal and are spaced apart by the diameter (D2) of the grooved rolls of the second stand (11a) and (11b), thereafter the end of the blank (17b) is guided into a hole (10) of an entry guide (9) of the second rolling stand, then the end of the blank (17b) is guided into the circular-shaped grooves (12a) and (12b), which are located on the cylindrical surfaces of the grooved rolls of the second stand (11a) and (11b), and the blank (17b) with an oval-shaped cross-section is flow formed into a bar (17c) with a nearly circular cross-section, wherein the diameter (dp) of the bar (17c) is greater than the diameter (dk) of the rolled ball (18), wherein behind the rolling gap of the second stand, the rolled bar (17c) is guided in a square-shaped hole (14) of a rear guide (13) of the second rolling stand, after which the rolled bar (17c) is moved in grooves (16a) and (16b) of the guide rollers (15a) and (15b) towards skew rolls (20a) and (20b), and the bar (17c) is guided into a hole of a feeding sleeve (19), in which the correct position of the bar (17c) is maintained, then, using the guide rollers (15a) and (15b), the bar (17c) is guided into a workspace of a skew rolling mill, consisting of two helical rolls (20a) and (20b) and two guides (24a) and (24b), wherein the both helical rolls (20a) and (20b) have the same working diameter (D), and their axes are twisted in opposite directions relative to the rolling axis by the same value of the twist angle of the rolls (γ), while the guides (24a) and (24b) are located parallel to the rolling axis, and the distance between the working surfaces of the guides (24a) and (24b) is greater than the diameter (dp) of the rolled bar (17e), then the end of the bar (17c) is gripped with conical surfaces (21a) and (21b) located in an entry zone of two helical rolls (20a) and (20b), which rotate with equal speeds (n5) in the same direction and the bar (17c) is set to rotate at a constant speed (n6) in the direction opposite to the direction of rotation of the helical rolls (20a) and (20b), and the cross-section of the bar (17c) is flow formed using conical surfaces (21a) and (21b), and the cross-section of the bar (17c) is calibrated to a diameter (d) smaller than the diameter of the rolled ball (dk) using two cylindrical surfaces (22a) and (22b) located behind the conical surfaces of the helical rolls (20a) and (20b), and subsequently, helical protrusions located on the surfaces of the helical rolls (20a) and (20b) are sunk into the cylindrical surface of the earlier calibrated bar (17c), wherein the helical protrusions of the helical rolls (20a) and (20b) have concave side surfaces (23a) and (23b), the radius (Rk) of which is equal to half the diameter (dk) of the rolled ball (18), and then, annular grooves with spherical side surfaces are gradually formed on the blank (17c), with the blank (17c) being held in the workspace during the rolling by two guides (24a) and (24b), located opposite each other, between the helical rolls (20a) and (20b), then, as a result of the action of the helical protrusions with the concave side surfaces (23a) and (23b) located on the helical rolls (20a) and (20b), the depth of the annular grooves increases until the ball (18) is formed and completely separated from the bar (17c), and as a result, the ball (18) with a diameter (dk) smaller than the diameter (dp) of the bar (30e) is obtained.
